

1

2,805,195

## ELECTROLYTIC MANGANESE

James H. Jacobs, Marietta, Ohio, and Michael C. Carosella, Niagara Falls, and James B. Culbertson, Lockport, N. Y., assignors to Union Carbide Corporation, a corporation of New York

No Drawing. Application April 2, 1956,  
Serial No. 575,313

2 Claims. (Cl. 204—105)

The present invention relates to an improved electrolytic manganese process and, more particularly, to a process employing electrolyte modifiers that control the formation of the deposited manganese metal.

In the production of metallic electrolytic manganese, the form of the deposited metal is of the greatest importance since it influences the efficiency of the process, the purity of the deposited metal, and the ease with which the deposited metal can be stripped from the cathode.

If the deposited metal is coarsely granular, it may build up on the cathode in small nodules that grow radially, forming a cauliflower-like structure from which electrolyte is not easily washed. Also, in this form the metal is not easily stripped from the cathode material (if this is not the same metal as that being deposited), since the metal tends to come off in individual nodules rather than in sheets or plates. In some processes, the deposited metal is removed from the cathodes by flexing or vibrating the latter; if the deposit is nodular, it tends to flex with the cathode and does not break loose.

Another difficulty encountered is "treeing"; that is, some nodules may grow at a much greater rate than the average, thus becoming much extended above the surface of the cathode deposit. In some cells this may make it mechanically difficult to remove the cathodes, or may upset current distribution (thus aggravating the condition). In addition, the nodules tend to be broken off and lost during handling, decreasing metal recovery.

A further difficulty encountered is the influence of cathode metal structure on deposition time. Obviously, if cathodes must be changed frequently, the overall process efficiency is greatly reduced. As mentioned above, treeing of the cathode metal, once started, becomes self-propagating and the extension or growth of the trees can be allowed to continue only to a limited extent before the cathode must be changed, even though the volume of deposited metal is far less than that physically permissible in the form of a thin, rectangular body. Therefore, the provision of any material in the electrolyte, which will prevent treeing and maintain formation of a relatively flat, smooth deposit, will greatly increase the efficiency of the overall electrowinning process.

Heretofore, various organic compounds, such as gums and glues, have been used in many processes as electrolyte additives to prevent the formation of nodular structures,

2

but these compounds are not equally effective with all processes.

It is an object of the present invention to extend the deposition time, and thus simplify and improve the efficiency of the process for the electrowinning of manganese by reducing the frequency at which cathodes must be removed, stripped, prepared and reinserted in cell.

Another object of the invention is to produce electrolytic manganese metal of improved purity.

10 A further object of the invention is to produce metallic manganese metal that is sound, dense, less friable and of greater thickness than otherwise obtained, and, therefore, easier to handle and use.

The electrowinning of some metals is much more easily 15 accomplished than others; copper, silver, and nickel may be electrodeposited without particular difficulty. One of the metals which is more difficult to obtain electrolytically is manganese which tends to deposit in irregular fashion and in nodular form, and is very prone to form trees. 20 Prior practice for electrowinning of manganese was such that not more than a 25- to 30-hour deposition period could be achieved. If it was attempted to continue deposition beyond this length of time, the quality of the metal degenerated and became unacceptable.

25 By the process of this invention, high-quality manganese metal can be electrodeposited for periods of two to four times as long as is possible with prior processes.

The present invention comprises a process for electrowinning of manganese from an electrolyte composed substantially of manganese sulphate, ammonium sulphate, and potassium sulphate which serves as a smoothing agent. The presence of specific quantities of potassium sulphate in the electrolyte has a marked effect upon the character of the manganese metal deposited at the cathode.

30 35 By the addition or other provision of potassium sulphate in the electrolyte, the character of deposited metal is altered from soft to dense, hard compact metal. This makes it possible to increase the continuous plating time by a factor of from two to four. Inclusion of potassium sulphate in the electrolyte has made it possible in some cases to obtain continuous deposition of dense, hard manganese metal for periods up to 72 and 96 hours, a far longer period than is possible in the absence of this addition agent, and appreciably longer than has been possible with any additive of the prior art.

40 45 As is well known in the art, a small amount of sulphur dioxide is added to the cell feed solution (in a concentration of about 0.1 to 1.0 gram per liter) to stabilize the solution and to increase the current efficiency.

50 55 More specifically, it has been found that the provision of between 20 and 70 grams per liter of potassium sulphate in the electrolyte will be effective in extending the deposition time without any sacrifice in current efficiency.

The data in the table below show that the progressive increase from 3.3 to 25 gms. per liter in the concentration of potassium sulphate in the cell feed over a 16-month period enabled the operators to extend the plating time by 50% with no drop in the current efficiency. This means that the plate is 50% thicker and that the appearance was good at the end of 72 hours.

| Run No. | Grams per Liter in Cell Feed |      |                                |                                                 | Current Effi- ciency | Plating Time, Hrs. | Appearance |
|---------|------------------------------|------|--------------------------------|-------------------------------------------------|----------------------|--------------------|------------|
|         | Mn                           | K    | K <sub>2</sub> SO <sub>4</sub> | (NH <sub>4</sub> ) <sub>2</sub> SO <sub>4</sub> |                      |                    |            |
| 1       | 31                           | 1.48 | 3.3                            |                                                 | 115                  | 61                 | 48         |
| 2       | 31                           | 1.72 | 3.8                            |                                                 | 118                  | 61                 | 48         |
| 3       | 30                           | 2.32 | 5.2                            |                                                 | 114                  | 62                 | 72         |
| 4       | 34                           | 3.60 | 8.0                            |                                                 | 120                  | 63                 | 48         |
| 5       | 34                           | 6.20 | 13.8                           |                                                 | 132                  | 62                 | 48         |
| 6       | 34                           | 6.5  | 14.5                           |                                                 | 137                  | 61                 | 48         |
| 7       | ( <sup>1</sup> )             | 8.0  | 17.8                           |                                                 | 136                  | 62                 | 48         |
| 8       | 35                           | 8.50 | 19.0                           |                                                 | 133                  | 65                 | 48         |
| 9       | 31                           | 9.75 | 21.8                           |                                                 | 133                  | 62                 | 72         |
| 10      | ( <sup>1</sup> )             | 10.7 | 23.8                           |                                                 | 128                  | 64                 | 72         |
| 11      | 33                           | 10.8 | 24.0                           |                                                 | 125                  | 63.6               | 72         |
| 12      | 32                           | 11.4 | 25.4                           |                                                 | 123                  | 63                 | 72         |
| 13      | ( <sup>1</sup> )             | 11.0 | 24.5                           |                                                 | 129                  | 63.5               | 72         |

<sup>1</sup> Not measured.<sup>2</sup> Medium base means a dense layer of medium thickness adjacent to the cathode. The product had built up on this base in the form of nodules.

The prime objective of the tests which yielded the above data was to produce thick plate of dense structure and smooth surface. For the same current efficiency the thickness of the plate is a direct function of the time. Therefore, the plating time was extended as long as was compatible with the production of dense plate having a minimum of "trees" or nodular structure. The data show that 48-hour plate was not uniformly good until the potassium sulphate concentration approached 20 gms. per liter of cell feed; also that the attempt to run 72 hours in run No. 3 was not successful because the surface appearance was not good enough. From run No. 9 on, the plate was dense and thick with 72-hour plating time and was essentially free of "trees" or nodular structure since the potassium sulphate concentration was increased from 21 to about 25 gms. per liter.

The upper limit of 70 gms. potassium sulphate per liter was chosen as being the limit of solubility in a synthetic cell feed produced from materials essentially free of sodium but containing ammonium sulphate and manganese sulphate in normal amounts. This limit is the maximum concentration of potassium sulphate compatible with the other constituents of the normal cell feed for the electrowinning of manganese, i. e., manganese and ammonium sulphates with sodium sulphate as an impurity and sulphur dioxide addition as known to the prior art. Experiments on the use of various concentrations of sodium sulphate in the absence of potassium have shown that this salt is neither harmful nor beneficial. Consequently, it is considered as an impurity but it has a marked effect on the solubility of potassium sulphate. It has not been determined as to when this concentration of sodium sulphate becomes critical.

However, early experiments showed that sodium sulphate 38 gms. per liter permitted a concentration of 30 gms. per liter of potassium sulphate (68 gms./l. total) in the standard cell feed. This was the maximum obtainable with this sodium concentration. Consequently, a figure of 70 gms. potassium sulphate per liter was specified as a practical top limit. This assumes that the concentration of potassium sulphate could easily reach this figure in the standard cell feed with a minimum of sodium sulphate present since potassium salts are generally speaking more soluble than sodium salts.

In an example of the process of the invention, an elec-

trolyte was continually electrolyzed to produce a catholyte containing about 11.0 grams per liter manganese, 128.5 grams per liter ammonium sulphate, 0.75 gram per liter sulphur dioxide, and 32 grams per liter potassium sulphate in the cathode compartment of a diaphragm electrolytic cell employing 99% lead-1% silver alloy anodes and stainless steel cathodes. The cathode current density employed was about 40 amperes per square foot and a catholyte pH of about 8.5 was maintained. Solid, dense manganese metal was deposited on the cathode for 48 hours before a fine nodular structure began to appear. There was no evidence of treeing or loss in current efficiency at any time during the deposition period.

This is a continuation-in-part of our copending application Serial No. 378,403 filed September 3, 1953, now abandoned.

What is claimed is:

40 1. In a process for the electrowinning of metallic manganese employing a diaphragm compartment cell and an electrolyte comprising an aqueous manganese and ammonium sulphate solution containing an amount of sulphur dioxide effective to stabilize the solution and increase 45 the current efficiency, the improvement which comprises providing and maintaining in said electrolyte solution during electrolysis between about 20 and 70 grams per liter of potassium sulphate, whereby a thick, dense metallic manganese deposit substantially free of nodules is produced.

50 2. A process for the electrowinning of metallic manganese employing a diaphragm compartment cell and an electrolyte comprising an aqueous manganese and ammonium sulphate solution containing an amount of sulphur dioxide effective to stabilize the solution and increase 55 the current efficiency comprising, providing in said cell an aqueous solution containing manganese sulphate, ammonium sulphate, sulphur dioxide, and between 20 and 70 grams per liter of potassium sulphate, and electrolyzing 60 said solution to form at the cathode of said cell, a thick, dense metallic manganese deposit substantially free of nodules.

65 References Cited in the file of this patent

UNITED STATES PATENTS

2,446,313 Vedensky ----- Aug. 3, 1948